



US007517060B2

(12) **United States Patent**  
Hess et al.

(10) Patent No.: US 7,517,060 B2  
(45) Date of Patent: Apr. 14, 2009

- |      |                                                                                                                                                     |               |         |                            |
|------|-----------------------------------------------------------------------------------------------------------------------------------------------------|---------------|---------|----------------------------|
| (54) | <b>FLUID-EJECTION DEVICES AND A DEPOSITION METHOD FOR LAYERS THEREOF</b>                                                                            | 4,708,915 A   | 11/1987 | Ogawa et al.               |
|      |                                                                                                                                                     | 4,828,935 A   | 5/1989  | Jonker et al.              |
|      |                                                                                                                                                     | 4,862,197 A   | 8/1989  | Stoffel                    |
| (75) | Inventors: <b>Ulrich E. Hess</b> , Corvallis, OR (US);<br><b>Samson Berhane</b> , Corvallis, OR (US);<br><b>Arjang Fartash</b> , Corvallis, OR (US) | 4,872,028 A   | 10/1989 | Lloyd                      |
|      |                                                                                                                                                     | 4,951,063 A * | 8/1990  | Hawkins et al. .... 347/62 |
|      |                                                                                                                                                     | 4,967,208 A   | 10/1990 | Childers                   |
|      |                                                                                                                                                     | 4,982,199 A   | 1/1991  | Dunn                       |

(73) Assignee: **Hewlett-Packard Development Company, L.P.**, Houston, TX (US)

( \*) Notice: Subject to any disclaimer, the term of this patent is extended or adjusted under 35 U.S.C. 154(b) by 329 days.

(21) Appl. No.: 11/345,755

(22) Filed: Feb. 2, 2006

### Prior Publication Data

US 2006/0125882 A1 Jun. 15, 2006

### Related U.S. Application Data

- (60) Division of application No. 10/620,666, filed on Jul. 16, 2003, now Pat. No. 7,025,894, which is a continuation-in-part of application No. 09/978,985, filed on Oct. 16, 2001, now abandoned.

(51) **Int. Cl.**  
**B41J 2/05** (2006.01)

(52) U.S. Cl. .... 347/64; 347/63; 347/62;  
347/61

(58) **Field of Classification Search** ..... 343  
347/56, 54, 62-65, 67, 202  
See application file for complete search history.

(56) **References Cited**

U.S. PATENT DOCUMENTS

- |           |     |         |                 |
|-----------|-----|---------|-----------------|
| 4,058,430 | A   | 11/1977 | Suntola et al.  |
| 4,339,762 | A   | 7/1982  | Shirato et al.  |
| 4,488,084 | A   | 12/1984 | Lindfors et al. |
| 4,513,298 | A   | 4/1985  | Scheu           |
| 4,532,530 | A * | 7/1985  | Hawkins .....   |

(Continued)

## FOREIGN PATENT DOCUMENTS

EP 0 729 834 A2 4/1996

(Continued)

#### OTHER PUBLICATIONS

J. Stephen Aden et al.; "The Third Generation HP Thermal Inkjet Printhead"; pp. 41-45; Hewlett-Packard Company Journal; Feb. 1994.

*Primary Examiner*—Matthew Luu  
*Assistant Examiner*—Henok Legesse

(57) **ABSTRACT**

A cavitation structure for a print head has a first dielectric layer overlying at least a first portion of a substrate. A second dielectric layer has a first portion overlying at least a second portion of the substrate and a second portion, different from the first portion of the second dielectric layer, overlying at least a portion of the first dielectric layer. A cavitation layer has a first portion in contact with the first dielectric layer and a second portion in lateral contact with the second portion of the second dielectric layer. A third dielectric layer is disposed on only the first portion of the second dielectric layer.

**15 Claims, 2 Drawing Sheets**



## U.S. PATENT DOCUMENTS

|               |         |                   |                 |         |                          |
|---------------|---------|-------------------|-----------------|---------|--------------------------|
| 5,083,137 A   | 1/1992  | Badyal et al.     | 6,046,758 A     | 4/2000  | Brown et al.             |
| 5,168,284 A   | 12/1992 | Yeung             | 6,065,823 A     | 5/2000  | Kawamura                 |
| 5,187,500 A   | 2/1993  | Bohorquez et al.  | 6,123,419 A     | 9/2000  | Cleland                  |
| 5,194,877 A   | 3/1993  | Lam et al.        | 6,126,276 A     | 10/2000 | Davis et al.             |
| 5,227,812 A   | 7/1993  | Wantanabe et al.  | 6,139,131 A     | 10/2000 | Prasad et al.            |
| 5,257,042 A * | 10/1993 | Buhler .....      | 6,287,965 B1 *  | 9/2001  | Kang et al. .... 438/648 |
| 5,294,286 A   | 3/1994  | Nishizawa et al.  | 6,293,654 B1    | 9/2001  | Pidwerbecki              |
| 5,357,081 A   | 10/1994 | Bohorquez         | 6,299,294 B1 *  | 10/2001 | Regan .....              |
| 5,418,558 A   | 5/1995  | Hock et al.       | 6,328,428 B1    | 12/2001 | Keefe et al.             |
| 5,428,376 A   | 6/1995  | Wade et al.       | 2002/0094663 A1 | 7/2002  | Kwon et al.              |
| 5,526,027 A   | 6/1996  | Wade et al.       |                 |         |                          |
| 5,530,465 A   | 6/1996  | Hasegawa et al.   | EP 0 750 990 A2 | 2/1997  |                          |
| 5,742,322 A   | 4/1998  | Cranton et al.    | EP 0 794 057 A1 | 10/1997 |                          |
| 5,883,650 A   | 3/1999  | Figueroedo et al. | EP 0 825 026 A2 | 2/1998  |                          |
| 5,916,365 A   | 6/1999  | Sherman           |                 |         |                          |
| 6,007,188 A   | 12/1999 | MacLeod et al.    |                 |         |                          |

## FOREIGN PATENT DOCUMENTS

|    |              |         |
|----|--------------|---------|
| EP | 0 750 990 A2 | 2/1997  |
| EP | 0 794 057 A1 | 10/1997 |
| EP | 0 825 026 A2 | 2/1998  |

\* cited by examiner



*Fig. 1*



*Fig. 2*



*Fig. 3*

**FLUID-EJECTION DEVICES AND A  
DEPOSITION METHOD FOR LAYERS  
THEREOF**

**CROSS REFERENCE TO RELATED  
APPLICATIONS**

This is a divisional application of application Ser. No. 10/620,666, titled "FLUID-EJECTION DEVICES AND A DEPOSITION METHOD FOR LAYERS THEREOF," filed Jul. 16, 2003 now U.S. Pat. No. 7,025,894, which is a Continuation-in-Part of U.S. application Ser. No. 09/978,985 filed Oct. 16, 2001 (abandoned), which applications are incorporated herein by reference.

**BACKGROUND**

Commercial products having imaging capability, such as computer printers, graphics plotters, facsimile machines, etc., have been implemented with fluid-ejection devices producing printed media. In many cases, such devices utilize inkjet technology whereby an inkjet image is created when a precise pattern of dots is formed on a printing medium from ejected ink droplets. Typically, an inkjet print head is supported on a movable carriage that traverses over the surface of the print medium and is controlled to eject drops of ink at appropriate times pursuant to commands of a microcomputer or other controller, wherein the timing of the application of the ink drops is intended to correspond to a pattern of pixels of the image being printed. A typical inkjet print head includes an array of precisely formed nozzles in an orifice plate. The plate is attached to a thin-film substrate that implements ink firing heater resistors and apparatus for enabling the resistors. The thin-film substrate is generally comprised of several thin layers of insulating, conducting, or semiconductor material that are deposited successively on a supporting substrate, or die, in precise patterns to form collectively, all or part of an integrated circuit.

The thin-film substrate or die is typically comprised of a layer, such as silicon, on which are formed various thin-film layers that form thin-film ink firing resistors, apparatus for enabling the resistors, and interconnections to bonding pads that are provided for external electrical connections to the print head. Ongoing improvements in the design of fluid-ejection devices have resulted in more efficient print-head components, such as resistors barrier layers, and passivation layers. In some cases, barrier layers and passivation layers deposited by physical vapor deposition or chemical vapor deposition methods have been utilized to improve performance. In other cases; sputtering techniques have been used to form barrier layers and passivation layers. While these techniques have some utility, it is desirable to have an improved barrier layers and passivation layers capable of improving performance and increasing resistor life.

Of course, energy expenditure is necessary for operation of fluid-ejection devices. In this regard, the term "turn-on energy" relates to the energy required to form a vapor bubble of a size sufficient to eject a predetermined amount of ink volume through a print head nozzle. With ever increasing usage of electrically driven devices, conservation becomes an important consideration. With respect to fluid-ejection devices, a reduction in "turn-on energy" would be desirable,

especially if such reduction produced improved print head performance and prolonged print head life.

**SUMMARY**

One embodiment of the present invention provides a method of forming a cavitation layer of a print head. The method includes utilizing an atomic layer deposition process.

**DESCRIPTION OF THE DRAWINGS**

FIG. 1 is a cross-sectional view of a portion of a fluid-ejection device according to an embodiment of the present invention.

FIG. 2 is a cross-sectional view of a portion of a fluid-ejection device according to another embodiment of the present invention.

FIG. 3 illustrates a passivation layer according to another embodiment of the present invention.

**DETAILED DESCRIPTION**

In the following detailed description of the present embodiments, reference is made to the accompanying drawings that form a part hereof, and in which is shown by way of illustration specific embodiments in which the invention may be practiced. These embodiments are described in sufficient detail to enable those skilled in the art to practice the invention, and it is to be understood that other embodiments may be utilized and that process, electrical or mechanical changes may be made without departing from the scope of the present invention. The following detailed description is, therefore, not to be taken in a limiting sense, and the scope of the present invention is defined only by the appended claims and equivalents thereof.

Embodiments of the present invention involve forming layers of fluid-ejection devices, such as print heads, using atomic layer deposition (ALD). ALD involves depositing a selected composition on crystalline or amorphous substrates or layers one molecular layer at a time. Unlike atomic layer epitaxy (ALE) processes that involve growing a single crystalline layer on a crystalline substrate or layer that mimics the substrate or layer, ALD does not require a crystalline substrate or layer, as does ALE. ALE operates in a ultra-high-to-high vacuum, e.g., corresponding to absolute pressures from about  $10^{-10}$  to about  $10^{-7}$  Torr, whereas ALD operates in medium-to-low vacuum, e.g., corresponding to absolute pressures from about  $10^{-3}$  to about 1 (one) Torr.

For one embodiment, a passivation layer is formed on a surface of a substrate. The passivation layer generally protects exposed elements of the fluid-ejection device from environmental contaminants, e.g., fluids, such as ink, thus ensuring electrical stability of the fluid-ejection device. For another embodiment, the passivation layer is a thin dielectric layer.

The passivation layer is deposited using the ALD process referred to herein as, for example, an ALD dielectric or an ALD passivation layer, as appropriate. In other embodiments, a cavitation layer of a firing chamber of the fluid-ejection device is formed using ALD and is referred to herein as an ALD cavitation layer, for example.

FIG. 1 is an unscaled cross-sectional view of a portion of a fluid-ejection device (or print head) 21 according to an embodiment of the present invention. The fluid-ejection device 21 is comprised of a plurality (or stack) of thin film layers, generally indicated by the reference numeral 26, that are stacked atop a die 49. Contact termination in the print head is also shown in FIG. 1, as described in more detail below.

The layers over the die **49** form thin-film ink firing resistors or heating elements, such as a resistive layer (or resistor) **48**, and an apparatus for enabling the resistors. In a particular embodiment, the die **49** (e.g., about 650 microns thick) is composed of silicon. The silicon die **49** is a semiconductor that functions as a substrate to support the overlying layers. In this regard, immediately overlying the die **49** there is formed by plasma enhanced chemical vapor deposition (PECVD) of a tetra ethyl ortho silicate (TEOS) or silane (SiH<sub>4</sub>) based oxide (e.g., about 1.0 micron thick) layer **47**. This layer insulates the overlying inkjet circuitry from the silicon die **49** and provides thermal isolation from the silicon, thereby keeping the circuitry above the layer **47** from being shorted out by the silicon below. In operation, the layer **47** functions as a stand-off so that heat moves away from, rather than toward, the silicon die **49**.

A layer **45**, formed by plasma enhanced chemical vapor deposition (PECVD) of one embodiment, is deposited upon the layer **47**. For another embodiment, layer **45** is formed by ALD and is about 250 angstroms thick. For one embodiment, layer **45** is a layer of an amorphous material, such as silicon nitride (Si<sub>3</sub>N<sub>4</sub>). The layer **45** chemically stabilizes the underlying TEOS-oxide layer **47** and provides thermal and chemical stabilization of resistive layer **48**. Resistive layer **48** is patterned on layer **45** and is chemically defined by an etching process. Layer **48** is comprised of resistive materials such as tantalum, aluminum, silicon, or tantalum nitride and it functions to resistively heat the overlying structure to enable ejection of an ink droplet.

The overlying structure includes a passivation layer **42** that is deposited, patterned, and etched to open up contact holes at end of the resistive layer **48**. Specifically, passivation layer **42** is deposited on layer **45** and layer **48** using ALD. Passivation layer **42** is structured to create interconnects to a layer **41** (e.g., about 0.5 micron thick). In one embodiment, the layer **41** is a thin tungsten film (e.g., about 0.5 micron thick) deposited and patterned by plasma processes. Overlying the tungsten layer **41** is a TEOS-oxide layer (e.g., about 0.6 micron thick) **39** that is disposed laterally in relation to the firing chamber **24**. The layer **39** is etched to enable an overlying aluminum contact terminal **35** to contact the tungsten layer **41**. In this manner, the layer **39** functions as an interdielectric between two metals, the underlying tungsten layer **41** and the overlying aluminum contact terminal **35**.

In the embodiment shown in FIG. 1, the firing chamber **24** includes a cavitation layer **31** deposited over the stack **26** and in contact laterally with a tetra ethyl ortho silicate (TEOS)-oxide layer (e.g., about 0.6 micron thick) **33**. The cavitation layer **31** provides mechanical protection to the underlying structure and, in particular, prevents chemical and impact damage to the resistor **48**. The TEOS layer **33**, on the other hand, provides insulation for the layers of the fluid-ejection device and separates the cavitation layer **31** from other structures. It will be noted that the cavitation layer **31** is isolated throughout the ejection device **21**, except where it contacts the ALD passivation layer **42**. Cavitation layer **31** can be of tantalum (Ta), titanium (Ti), molybdenum (Mo), niobium (Nb), etc. For one embodiment, cavitation layer **31** is deposited on layer **33** and layer **42** using ALD. For another embodiment cavitation layer **31** is about 500 angstroms thick. Using ALD for cavitation layer **31** results in conformal coverage over layer **33** and produces a low-stress, substantially crack-free film.

For some embodiments, a passivation layer **110** is disposed on layer **33** using ALD, chemical vapor deposition, or the like. For one embodiment, passivation layer **110** is a carbide layer, such as SiC silicon carbide, diamond like carbons (DLCs),

e.g., fullerenes or graphite, etc. Passivation layer **110** acts to protect layer **33** against inks and other fluids. Passivation layer **110** also acts to protect against wear.

In one embodiment, the passivation layer **42** is a dielectric film, such as silicon carbide, diamond like carbon, aluminum oxide etc. For one embodiment, passivation layer **42** has a thickness of between about 250 angstroms and 2000 angstroms. For another embodiment, passivation layer **42** has a thickness between about 250 to 500 angstroms, preferably about 300 angstroms. This thin film enables substantially reduced drive energies because of the thinness of the dielectric and, possibly, because of enhanced thermal conductivity. Dielectrics that can be deposited by the ALD technique contain refractory metals, transitional metals, and insulators, such as silicates. Other dielectrics depositable by atomic level deposition include metal oxides, nitrides, borides, and carbides.

Examples of oxides depositable by atomic level deposition include aluminum oxide (Al<sub>2</sub>O<sub>3</sub>), titanium oxide (TiO<sub>2</sub>), tantalum oxide (Ta<sub>2</sub>O<sub>5</sub>), hafnium oxide (HfO<sub>2</sub>), magnesium oxide (MgO), cesium oxide (CeO<sub>2</sub>), niobium oxide (Nb<sub>2</sub>O<sub>5</sub>), lanthanum oxide (La<sub>2</sub>O<sub>3</sub>), yttrium oxide (Y<sub>2</sub>O<sub>3</sub>), aluminum titanium oxide (Al<sub>x</sub>Ti<sub>y</sub>O<sub>z</sub>), tantalum hafnium oxide (Ta<sub>x</sub>Hf<sub>y</sub>O<sub>z</sub>), etc. Examples of nitrides depositable by atomic level deposition include silicon nitride (SiN), aluminum nitride (AlN), titanium nitride (TiN), tantalum nitride (TaN), niobium nitride (NbN), molybdenum nitride (MoN), tungsten nitride (WN), etc. Examples of refractory metals depositable by atomic level deposition include tantalum (Ta), titanium (Ti), tungsten (W), molybdenum (Mo), niobium (Nb), titanium nitride (TiN), tantalum nitride (TaN), niobium nitride (NbN), molybdenum nitride (MoN), tungsten nitride (WN), etc. Examples of transitional metals depositable by atomic level deposition include tantalum (Ta), titanium (Ti), tungsten (W), copper (Cu), molybdenum (Mo), hafnium (Hf), etc. Examples of borides depositable by atomic level deposition include titanium diboride (TiB<sub>2</sub>), zirconium diboride (ZrB<sub>2</sub>), arsenic hexaboride (AsB<sub>6</sub>), etc.

During the ALD process, a source-material precursor and a binding precursor are employed alternately with inert purge gasses in between. The purge gasses ensure that no stray gasses, such as the source-material precursor, are present before the next gas, such as the binding precursor, is employed. The deposited source-material precursor chemically reacts on the surface with the deposited binding precursor to form a single molecular ALD layer. The single molecular ALD layers build up molecular layer-by-molecular layer using this process. As a result of the monolayer-by-monolayer build up, the final thickness of the ALD layer is well controlled.

Examples of source-material precursors include trimethylated aluminum (Al(CH<sub>3</sub>)<sub>3</sub>), aluminum trichloride (AlCl<sub>3</sub>), titanium tetrachloride (TiCl<sub>4</sub>), tantalum pentachloride (TaCl<sub>5</sub>), bis(tert-butylimido), bis(dimethylamido)tungsten ((BuN)<sub>2</sub>(Me<sub>2</sub>N)<sub>2</sub>W), methane (CH<sub>4</sub>), etc. Examples of binding precursors include oxygen-source materials, e.g., water vapor, a nitrogen-source materials, e.g., ammonia, hydrogen, etc.

For one embodiment, the source-material precursors include a dopant, such as aluminum, nitrogen, carbon, oxygen, etc. For this embodiment, the ALD process is used to deposit layers that include the dopant. For another embodiment, the ALD process is used to deposit a cavitation layer **31** with a dopant. For some embodiments, the dopant, e.g., nitrogen or the like, reduces a thermal resistance of cavitation layer

31. This acts to reduce the thermal resistance between resistive layer **48** and ink contained in firing chamber **24**, resulting in a lower turn-on energy.

For another embodiment, the ALD process is used to deposit a passivation layer **42** that includes a dopant, such as aluminum, boron, phosphorous, germanium, barium, calcium, strontium, etc., for reducing the thermal resistance of layer **42**, which acts to reduce the thermal resistance between resistive layer **48** and ink contained in firing chamber **24**. For other embodiments, adding a dopant to layer **42**, e.g., carbon, oxygen, etc., acts to increase the thermal resistance of layer **42**. For other embodiments, dopants such as phosphorous, oxygen, carbon, nitrogen, etc., act to increase the hardness, reduce plastic flow, etc. of the respective layer.

For some embodiments, a seed layer **115**, e.g., of tungsten, titanium nitride, or tantalum nitride is deposited on ALD passivation layer **42** using ALD and layer **41** is subsequently formed on seed layer **115**. For other embodiments, a seed layer **120**, e.g., of titanium nitride or tantalum, is deposited on layer **39** using ALD and aluminum contact terminal **35** is subsequently formed on seed layer **120**. For various embodiments, seed layers **115** and **120** are about 100 angstroms thick.

FIG. 2 is an unscaled cross-sectional view of a fluid-ejection device **221** according to another embodiment of the present invention. The device **221** is comprised of a plurality (or stack) of thin-film layers, generally indicated by the reference numeral **226**. The device **221** utilizes ALD layers, and utilizes contact termination as described above in reference to the ejection device **21**. The fluid-ejection device **221** includes a firing chamber **224**. In addition, the fluid-ejection device **221**, like the device **21** of FIG. 1, is comprised of a plurality of thin-film layers stacked on a silicon die **65**.

The die **65** is similar in structure and function to the die **49** of FIG. 1. A field oxide or TEOS layer (e.g., about 1.0 micron thick) **63**, similar in structure and function to the layer **47** of FIG. 1, is disposed on the die **65** and a heating (or resistor) layer **57**, composed of tantalum/aluminum, or other suitable metal, is disposed on the layer **63**. An aluminum layer (e.g., about 0.5 micron thick) **55** is disposed laterally of a region **228** of firing chamber **224** and overlying the layer **57**. The aluminum layer **55** is covered by an ALD dielectric (e.g., about 0.1 micron thick) film **52**. The ALD film **52** is similar to the layer **42** of FIG. 1 and is formed according to the above-described process. For other embodiments, layer **52** is similar to and is formed as described for layer **10** of FIG. 1.

Firing chamber **224** includes a cavitation layer **51** deposited over the stack **226**. For one embodiment, cavitation layer **51** is deposited on layer **33** using ALD. Cavitation layer **51** can be of tantalum (Ta), titanium (Ti), molybdenum (Mo), niobium (Nb), etc. For another embodiment cavitation layer **51** is about 500 angstroms thick. For one embodiment, a seed layer **230**, e.g., of refractory metal, is deposited on layer **57** using ALD, and layer **55** is subsequently formed on seed layer **230**. For some embodiments, seed layer **230** is about 100 angstroms thick.

For some embodiments, the passivation layers of the present invention, such as passivation layers **42** and **110** of FIG. 1 and passivation layer **52** of FIG. 2 include multiple layers as is shown generally for a passivation layer **300** in FIG. 3. For one embodiment, passivation layer **300** includes layers **310<sub>1</sub>** to **310<sub>N</sub>**. For another embodiment, each of layers **310<sub>1</sub>** to **310<sub>N</sub>** is formed using ALD, chemical vapor deposition (CVD) or the like and has a thickness between about 250 angstroms and about 350 angstroms. For another embodiment, some of the layers **310** are formed using ALD and others are formed using CVD, for example. For one embodiment, some of the layers **310** are of one material, such as silicon carbide and others are of another material, such as silicon nitride. For another embodiment, passivation layer **300** includes two layers, e.g., one of silicon nitride the other of silicon carbide.

ment, some of the layers **310** are of one material, such as silicon carbide and others are of another material, such as silicon nitride. For another embodiment, passivation layer **300** includes two layers, e.g., one of silicon nitride the other of silicon carbide.

The present invention affords several distinct advantages. Because the ALD passivation layers are so thin, they permit reduced drive energies with consequent low turn on energy drop generation of the resistor, for example, in the resistor regions of the ejection devices **21** and **221**. This, in turn, results in faster thermal response, thereby enabling a higher frequency of operation. The present invention enables rapid print head resistor heating and cool down. As a result, a thermally more efficient print head is achieved with resulting swath size increases. Such increases, in turn, substantially improve fluid-ejection device throughput.

In another embodiment, the invention affords the flexibility of using very thin multiple dielectrics for custom tailoring of thermal properties. This is because the ALD process enables addition of a single molecular layer at a time, a dielectric film having a precise predetermined thickness can be achieved.

A possible limitation of ALD is low growth rate that may lead to potential problems in mass production. Thus, ALD may not be able to compete with other widely used thin film deposition techniques, such as chemical vapor deposition (CVD) or physical vapor deposition (PVD).

Advantageously, however, the films produced by the ALD technique have low stresses and are substantially free of voids, pinholes, and cracks. These attributes of ALD films act to increase resistor life and print head life.

Because the chemical purity is very high, resistor printing and storage life are substantially extended. The high thermal efficiency of the present invention translates into comparatively lower steady state die temperatures and enhanced resistor life.

It is known by those skilled in the art that electrical shorts reduce yield in some fluid-ejection devices. In the embodiments described above, high particle tolerance in passivation is achieved. Thus, the likelihood of shorts is diminished thereby raising circuit yield.

## CONCLUSION

Although specific embodiments have been illustrated and described herein, it will be appreciated by those of ordinary skill in the art that any arrangement that is calculated to achieve the same purpose may be substituted for the specific embodiments shown. Many adaptations of the invention will be apparent to those of ordinary skill in the art. Accordingly, this application is intended to cover any adaptations or variations of the invention. It is manifestly intended that this invention be limited only by the following claims and equivalents thereof.

What is claimed is:

1. A cavitation structure for a print head, comprising:  
a first dielectric layer overlying at least a first portion of a substrate;  
a second dielectric layer having a first portion overlying at least a second portion of the substrate and a second portion, different from the first portion of the second dielectric layer, overlying at least a portion of the first dielectric layer;  
a cavitation layer having a first portion in contact with the first dielectric layer and a second portion in lateral contact with the second portion of the second dielectric layer; and

a third dielectric layer disposed on only the first portion of the second dielectric layer, such that an entire upper surface of the cavitation layer is free of the third dielectric layer;

wherein a first sidewall of the cavitation layer is in contact with a sidewall of a first portion of the third dielectric layer and a second sidewall of the cavitation layer is in contact with a sidewall of a second portion of the third dielectric layer.

2. The cavitation structure of claim 1, wherein at least one of the first dielectric layer, the cavitation layer, and the third dielectric layer is formed by atomic layer deposition.

3. The cavitation structure of claim 1, wherein at least one of the first and third dielectric layers is a carbide layer.

4. The cavitation structure of claim 1, wherein the first dielectric layer comprises a plurality of first dielectric layers, wherein at least one of the plurality of first dielectric layers is a silicon carbide layer and at least another of the plurality of first dielectric layers is a silicon nitride layer.

5. The cavitation structure of claim 1, wherein the cavitation layer is tantalum, titanium, molybdenum, or niobium.

6. The cavitation structure of claim 1, wherein the first and third dielectric layers are passivation layers.

7. A fluid ejection device, comprising:

a first dielectric layer overlying at least a first portion of a substrate;

a second dielectric layer having a first portion overlying at least a second portion of the substrate and a second portion, different from the first portion of the second dielectric layer, overlying at least a portion of the first dielectric layer;

a cavitation layer overlying the first dielectric layer and in lateral contact with the second portion of the second dielectric layer;

a third dielectric layer disposed on only the first portion of the second dielectric layer such that an entire upper surface of the cavitation layer is free of the third dielectric layer; and

a heating element interposed between the first dielectric layer and the substrate;

wherein a first sidewall of the cavitation layer is in contact with a sidewall of a first portion of the third dielectric layer and a second sidewall of the cavitation layer is in contact with a sidewall of a second portion of the third dielectric layer.

8. The fluid-ejection device of claim 7, wherein the first dielectric layer contains at least one of refractory metals, transitional metals, insulators, metal oxides, nitrides, borides, and carbides.

9. The fluid-ejection device of claim 7, wherein the third dielectric layer is of a diamond-like carbon or a silicon carbide.

10. The fluid-ejection device of claim 7, wherein at least one of the cavitation layer and the first dielectric layer comprises a dopant.

11. The fluid-ejection device of claim 7, further comprising one or more electrical contacts interposed between the first portion of the second dielectric layer and the second portion of the substrate.

12. A print head comprising:  
a first passivation layer overlying at least a first portion of a substrate;  
a dielectric layer having a first portion overlying at least a second portion of the substrate and a second portion, different from the first portion of the dielectric layer, overlying at least a portion of the first passivation layer;  
a cavitation layer overlying the first passivation layer and in lateral contact with the second portion of the dielectric layer;

a second passivation layer disposed on only the first portion of the dielectric layer such that an entire upper surface of the cavitation layer is free of the second passivation layer;

a heating element interposed between the first passivation layer and the substrate; and  
one or more electrical contacts interposed between the first portion of the dielectric layer and the second portion of the substrate;

wherein a first sidewall of the cavitation layer is in contact with a sidewall of a first portion of the second passivation layer and a second sidewall of the cavitation layer is in contact with a sidewall of a second portion of the second passivation layer.

13. The print head of claim 12, wherein the first passivation layer comprises a plurality of dielectric layers.

14. The print head of claim 12, wherein the second passivation layer is of a diamond-like carbon or a silicon carbide.

15. The print head of claim 13, wherein at least one of the plurality of dielectric layers of the first passivation layer is of silicon carbide and at least another of the plurality of dielectric layers is of silicon nitride.

\* \* \* \* \*

UNITED STATES PATENT AND TRADEMARK OFFICE  
**CERTIFICATE OF CORRECTION**

PATENT NO. : 7,517,060 B2  
APPLICATION NO. : 11/345755  
DATED : April 14, 2009  
INVENTOR(S) : Ulrich E. Hess et al.

Page 1 of 1

It is certified that error appears in the above-identified patent and that said Letters Patent is hereby corrected as shown below:

In column 5, line 46, delete "layer 10" and insert -- layer 110 --, therefor.

Signed and Sealed this

Fifteenth Day of September, 2009



David J. Kappos  
*Director of the United States Patent and Trademark Office*